

April 18, 1933.

C. DREYFUS

1,903,960

FABRIC AND SHEET MATERIAL AND THE MANUFACTURE THEREOF

Filed Dec. 15, 1925



INVENTOR  
CAMILLE DREYFUS  
BY  
*Bacchus & Wright*  
ATTORNEYS

Patented Apr. 18, 1933

1,903,960

# UNITED STATES PATENT OFFICE

CAMILLE DREYFUS, OF NEW YORK, N. Y.

## FABRIC AND SHEET MATERIAL AND THE MANUFACTURE THEREOF

Application filed December 15, 1925, Serial No. 75,653, and in Great Britain January 23, 1925.

This invention concerns the manufacture of new fabrics or sheet materials having waterproof to gas-proof properties or capable of other applications.

5 According to the invention, a fabric or sheet material is made by uniting under appropriate conditions of temperature and pressure, woven, knitted or other fabric composed of or containing filaments or fibers of thermoplastic cellulose derivative or derivatives with woven, knitted or other fabric composed of or containing filaments or fibers of non-thermoplastic or relatively non-thermo-  
10 plastic material.

15 According to the invention woven, knitted or other fabric made of yarns composed of filaments or fibers of a thermoplastic cellulose derivative, such for example as cellulose acetate, ethyl-, methyl- or benzyl-cellulose, nitro-cellulose or other ester or ether of cellulose, or mixtures of such cellulose derivatives, is associated with woven, knitted, or other fabric made wholly or partly of yarns composed of filaments or fibers of a non-thermo-  
20 plastic or relatively non-thermoplastic material, such for example as silk, cotton, linen, artificial filaments or fibers of the cellulose type, or wool or mixtures of any of such non-thermoplastic filaments or fibers with each  
25 other or it may be with filaments or fibers of a thermoplastic cellulose derivative or derivatives, and the associated fabrics are subjected to heat and pressure, with or without employment, assistance or application of plasticizing or softening agents or solvents of the thermoplastic cellulose derivative or derivatives; in this way the fabrics are united together and a composite sheet material is ob-  
30 tained in which the pores or interstices are re-  
35 duced to extremely minute dimensions, or closed completely, by the melting or softening effect produced by the heat and pressure upon the filaments and fibers of the thermoplastic cellulose derivative or derivatives and by the uniting of the fabrics under the heat and pressure. Two of such fabrics, i. e., one of each of the two classes specified above, may be associated and united together as referred to,  
40 45 50

with each other. Thus for example a fabric of cotton or composed of or containing other non-thermoplastic fiber may be disposed between two fabrics of cellulose acetate or other thermoplastic yarns; or a fabric of thermoplastic yarns may be disposed between two fabrics of cotton or composed of or containing other non-thermoplastic fibers; or four fabrics, two of each class, may be disposed so that the fabrics of thermoplastic yarn alternate respectively with the fabrics of cotton or composed of or containing other non-thermoplastic fibers, and so on.

55 The extent of the melting or softening effect, degree of closing the pores or interstices, and intimacy of union of the fabrics, and therefore the degree of impermeability of the compound fabric or material produced, can vary with the degrees and duration of heat and pressure employed, and with whether plasticizers, or softeners or solvents are employed, and with the number of fabrics united together, or other circumstances.

60 Thus for example the heat and pressure (with or without employment or assistance of plasticizing or softening agents or solvents) may be such as to unite the fabrics together and close or reduce to minute dimensions the pores or interstices of the compound or combined fabric and render the same water-resisting or even gas-resisting, without causing the filaments or fibers of the thermoplastic cellulose derivatives to disappear. Or the heat and pressure may be such as to cause the filaments or fibers of thermoplastic cellulose derivatives to melt and disappear partly or entirely.

65 It is to be understood that the degrees and duration of heat and pressure are interdependent and that all or any of these conditions may be varied according to circumstances or requirements. For example, the less the heat, the greater or longer is the pressure required to produce a given effect or vice versa; or again, the same conditions of heat and pressure may be applied for more or less time to produce the effect in a more or less pronounced degree.

70 75 80 85 90 95 100 The degree of the melting effect, and the degree of intimacy of union of the com-  
any desired relative number in alternation

uent fabrics, may be increased or accentuated by the employment, assistance or application of plasticizing or softening agents or solvents of the thermo-plastic cellulose derivative or derivatives as referred to, and it is to be understood that such agents or solvents, may be applied to or incorporated in any or all of the component fabrics before the application of the heat and pressure to the associated fabrics, for example, by the application of such agents or solvents in solution in volatile solvents thereof that are not solvents of the cellulose derivative or derivatives, and that alternatively, such agents or solvents may be incorporated in the filaments or fibers of thermoplastic cellulose derivatives in the production thereof, for example by employing such agents in the spinning solutions from which they are made.

Any plasticizing or softening agents or solvents, (preferably high-boiling or relatively high-boiling), of the cellulose derivatives may be employed. As some instances there may be mentioned triacetin, paratoluene sulphonamide or its derivatives, diethylphthalate, paratoluene sulphonanilide, and high-boiling alkylated xylene sulphonamide derivatives or preparations (for example, monomethyl xylene sulphonamide).

As the melting or softening effect is increased or accentuated by the plasticizing or softening agents or solvents, one can employ less heat and/or pressure for the production of a given effect when such agents or solvents are employed.

The invention is particularly applicable when fabric of cellulose acetate yarns is used as the component thermoplastic fabric of the compound fabric or material, and will hereinafter be described in this connection, it being understood, however, that fabrics of other cellulose esters or cellulose ethers may be employed as before indicated.

The heat and pressure may be applied in any appropriate way to the associated fabrics to be united together, for example by passage between pressure rollers, one or both of which is or are heated, or between a heated roller and a heated or cold plate or surface, or by pressure between heated plates or surfaces or between a heated plate or surface and a cold plate or surface, or by passing the associated fabrics under tension over a single heated roller, e. g. a calender roller, or by any other suitable means. In cases where the associated fabrics are passed through pairs of pressure rollers, the rollers in each pair may rotate at the same or at different speeds. Where the fabrics are passed under tension over a single heated roller, the roller may with advantage be rotated in an opposite direction to the travel of the fabric.

The manner in which the invention may

be carried into effect can be illustrated by the following more detailed description, it being understood that this can be varied widely without departing from the invention.

A woven or warp knitted fabric made of cellulose acetate yarn is associated with woven or knitted fabric of silk, cotton, linen or other fiber, preferably after being coated or treated with a plasticizing or softening agent or solvent on the face that is to contact with the latter fabric, and the associated fabrics are subjected to heat and pressure to unite the component fabrics together and give a material possessing a desired degree of resistance to penetration by water or gases, according to the degree and duration of temperature and pressure, the conditions of heat, pressure and time being interdependent. The less the heat, the greater or the longer is the pressure required to produce a given effect, or the same conditions of heat and pressure may be applied for more or less time to produce the effect in a greater or less degree.

Thus for example the associated fabrics (preferably with the cellulose acetate fabric treated with a plasticizing or softening agent or solvent) may be passed between heated pressure rollers, as in a calender, the conditions of heat, pressure and time being interdependent as before mentioned. For instance the associated fabrics may be passed slowly through heated calender rollers at temperatures between about 100° and 180° C. under pressures of from about 300 to 600 lbs. or more per square inch, according to the degree of melting or softening effect on the yarns of the cellulose acetate fabric and the degree of impermeability desired in the resulting compound material. The fabrics may be passed repeatedly between the heated rollers if desired, according to the degree of effect required.

Or again the associated fabrics may be passed once or repeatedly between a heated roller and a cold roller or platen, or they may be pressed between heated plates or between a heated plate and a cold platen. Or the heat and pressure may be applied in any other suitable way.

The application of plasticizing or softening agents or solvents of the cellulose acetate or other thermoplastic cellulose derivatives to assist the melting effect and the union of the component fabrics as hereinbefore referred to is especially of advantage where a high degree of impermeability to water is desired or for obtaining gas proof properties in the compound material. By way of example cellulose acetate fabric may be first treated with small quantities of water-insoluble, non-volatile plasticizers, softeners or solvents of cellulose acetate before being associated with the other fabric for subjection to the heat and pressure. These quantities may vary

for instance from about 1% to about 30% of the total quantity of cellulose acetate in the fabric, but more or less may be employed. The non-volatile plasticizers, softeners or solvents may be applied by spraying, dipping or otherwise, dissolved in a volatile solvent which does not dissolve the cellulose acetate, or in any other convenient way. Any suitable plasticizers, softeners or solvents and 10 any suitable volatile vehicle therefor may be used. As one example monomethylxylene sulphonamide may serve as a plasticizer and benzol as a vehicle, a suitable proportion being for instance about 20 grams of the sulphonamide dissolved in 100 grams of benzol for each 100 grams of cellulose acetate fabric. When the volatile solvent of the plasticizer or softener evaporates, the plasticizer or softener remains distributed evenly on the cellulose acetate fabric so that when this is associated with the other fabric and subjected therewith to the heat and pressure, it assists the melting or softening effect on the cellulose acetate yarns and the union of the component fabrics and closing of the pores or interstices of the component fabrics, thereby producing a compound material having waterproof to gasproof properties according to the degree of dissolving or melting effect etc, 20 produced on the cellulose acetate by the conditions of heat, pressure and time employed.

Instead of employing for association with fabric composed of yarns of thermoplastic filaments or fibers, fabric consisting wholly of yarns of silk, cotton or other non-thermoplastic fibers or filaments, one may employ for association therewith "mixed" fabric consisting of a mixture of thermoplastic yarns with yarns of silk, cotton, linen, artificial silk 30 of the cellulose type, wool or other non-thermoplastic fibers or filaments, or consisting of or comprising yarns composed of a mixture of thermoplastic filaments or fibers with non-thermoplastic fibers or filaments. Or one 40 may even, though with less advantage, employ only such mixed fabrics for making the compound material under the effect of heat and pressure, with or without application of plasticizing or softening agents or solvents, 45 the heat and pressure causing more or less melting or softening of the thermoplastic yarns, filaments or fibers and uniting the component fabrics together to form a compound material possessing greater or less degrees of 50 resistance to penetration by water or even gases, according to the temperature, pressure and duration of pressure or other conditions.

While fabrics made with yarns or fibers of nitrocellulose filaments or fibers may be 60 employed in practising the invention this is less advantageous owing to the inflammability of nitrocellulose.

The compound materials made according to the invention may be employed more 65 particularly for applications where resist-

ance to penetration by water or gases is desired, for instance as waterproof materials for garments, coverings, etc. or as materials for airships or other gas containers, but materials made according to the invention may be employed for any other technical or industrial applications.

For a further understanding of my invention reference is made to the accompanying drawing.

In this drawing Figure 1 shows the fabric 1 consisting wholly of yarns of a thermoplastic derivative of cellulose superposed upon the fabric 2 consisting of cotton yarns. After the two fabrics are pressed at elevated temperature in accordance with my invention, a sheet such as shown in Figure 2 is formed, wherein a more or less impervious layer 1a of the thermoplastic derivative adheres to the cotton fabric 2a.

In Figure 3 there are shown three layers of fabric, the middle fabric consisting of yarns of a thermoplastic derivative of cellulose such as cellulose acetate. In this figure a cotton fabric 3 is placed on the fabric 4 made of cellulose acetate yarns which in turn is placed over the cotton fabric 5. After these fabrics have been pressed in accordance with my invention, a composite sheet of fabric such as shown in Figure 4 is formed, wherein the intermediate layer 4a is a more or less impervious sheet of cellulose acetate between the cotton fabrics 3a and 5a.

In Figure 5 there are shown three layers of fabric in which the middle one is cotton while the outer fabrics are made of a thermoplastic derivative of cellulose yarn. The fabrics made of cellulose acetate are indicated at 6 and 8 while the cotton fabric is indicated at 7. After pressing these layers in accordance with my invention, a product shown in Figure 6 is produced wherein the cotton fabric 7a has an upper layer 6a and a lower layer 8a of more or less impervious cellulose acetate thereon.

In Figure 7 is shown a fabric 9 having yarns of cotton and also yarns of thermoplastic derivative of cellulose superposed upon a fabric 10 consisting wholly of silk yarns. After pressing in accordance with my invention a material shown in Figure 8 is formed wherein the silk fabric 10a has thereon a more or less impervious sheet 9a which has cotton yarns imbedded therein.

In Figure 9 there is shown a plan view of a mixed fabric containing yarns 12 of a thermoplastic derivative of cellulose such as cellulose acetate and yarns 11 of cotton. This sort of fabric may be used as the fabric 9 in Figure 7, or it may be pressed alone in accordance with my invention to form a more or less impervious film or thermoplastic derivative of cellulose in which cotton yarns are imbedded.

Having now particularly described and

ascertained the nature of my said invention and in what manner the same is to be performed, I declare that what I claim is:

1. A process for the manufacture of composite sheet material which comprises applying to a fabric containing yarns comprising a thermoplastic derivative of cellulose a softening agent in solution in volatile solvents which are non-solvents of said derivative, associating it with another fabric by superposition, and subjecting the fabrics to heat and pressure to soften the cellulose derivative and unite the fabrics to form a sheet material of increased impermeability.
- 10 2. A composite sheet material comprising a plurality of fabrics, at least one of which contains yarns comprising a thermoplastic derivative of cellulose, which fabrics have been united into a single sheet of relatively increased impermeability by the application of heat and pressure.
- 15 3. A process for the manufacture of composite sheet material which comprises applying to a fabric containing yarns comprising cellulose acetate a softening agent in solution in volatile solvents which are non-solvents of said cellulose acetate, associating it with another fabric by superposition, and subjecting the fabrics to heat and pressure
- 20 30 to soften the cellulose acetate and unite the fabrics to form a sheet material of increased impermeability.
- 35 4. A composite sheet material comprising a plurality of fabrics at least one of which contains yarns comprising cellulose acetate which fabrics have been united into a single sheet of relatively increased impermeability by the application of heat and pressure.

In testimony whereof, I have hereunto  
40 subscribed my name.

CAMILLE DREYFUS.